

Feb. 5, 1957

R. A. MACKE ET AL

2,780,581

PRODUCTION OF LUBRICATING OILS

Filed Sept. 29, 1954



INVENTORS.  
Edward F. Wadley,  
Robert A. Macke,  
BY

*John P. Mullin*  
ATTORNEY.

1

2,780,581

## PRODUCTION OF LUBRICATING OILS

Robert A. Macke and Edward F. Wadley, Baytown, Tex., assignors, by mesne assignments, to ESSO Research and Engineering Company, Elizabeth, N. J., a corporation of Delaware

Application September 29, 1954, Serial No. 459,059

2 Claims. (Cl. 196—14.42)

This invention concerns a novel process for producing lubricating oils of particularly high quality. The invention comprises a combination process for upgrading lubricating oil components of refinery stocks. In particular the invention concerns production of high viscosity index lubricating oils from paraffinic base crude oils and from cycle stocks resulting from the catalytic cracking of petroleum oils. It is the particular feature of this invention to produce lubricating oils by the solvent extraction of a mixture of catalytic cycle stock and paraffinic lubricant fractions. This process is particularly attractive in maximizing the yield of high quality lubricating oil from these lubricant sources.

As is generally known, an important criterion of a lubricating oil relates to the viscosity characteristics of the oil. For many applications, temperatures at which a lubricant must be employed are several hundred degrees Fahrenheit above temperatures existent prior to use of the lubricated mechanism. Consequently, it becomes a real problem to provide lubricating oils having the proper viscosity over the entire operating temperature range due to the decrease in viscosity of a lubricating oil as the oil becomes heated. This characteristic of a lubricating oil is generally identified as the "viscosity index" of the oil and essentially provides information as to the change in viscosity of the oil over the temperature range of 100 to 210° F. The higher the "viscosity index," the smaller the change in viscosity with temperature. It is apparent that for many applications it is desirable to employ lubricating oils having the highest possible viscosity index.

Production of high viscosity index lubricating oils can most readily be achieved by producing such lubricating oils from paraffinic base crude petroleums. Of all hydrocarbon types, paraffinic hydrocarbons have the highest viscosity indices falling in the range of about 125 to 180. Consequently, when the lubricating oil fraction is segregated from a paraffinic base crude oil it is relatively easy to process this fraction to obtain a final lubricating oil product having a high viscosity index. For example, the lubricating oil fraction of a paraffinic base crude oil can be treated with a selective solvent for aromatic hydrocarbons so as to provide a raffinate product of high viscosity index in relatively large yields. Paraffinic base crude oils particularly attractive for production of lu-

2

bricating oils include Panhandle, Ellenberger, New Hope, and Mid-Continent petroleums.

However, truly paraffinic lube crude oils are unusual at the present time, and the supply of such oils is limited.

5 The need, therefore, exists for extending available sources of feed stock for producing high viscosity index lubricating oils.

It has recently been found that high viscosity lubricating oils can be derived by processing steps applied to 10 mixed base crude oils. In accordance with the technique referred to, a gas oil fraction is segregated from a mixed base crude oil and subjected to a catalytic cracking operation. Thereafter the products of catalytic cracking, or that fraction of the products boiling in the lubricating oil 15 boiling range, are subjected to solvent extraction in order to recover a raffinate product rich in paraffinic materials and constituting a good lubricating oil base stock. The process of producing lubricating oils from the products of a catalytic cracking process in this manner is specifically 20 disclosed and claimed in United States Patent 2,660,552, issued November 24, 1953, to Forrest H. Blanding.

While the recovery of lubricating oils from catalytically cracked products is a particularly desirable and attractive process, the process is characterized by one disadvantage.

25 This is the fact that relatively low yields of high quality lubricating oil are obtained by the selective solvent extraction operation as compared to the yields which can be obtained by selective solvent extraction of paraffinic base lubricating oil distillates. For example, under comparable

30 conditions, solvent extraction of a Panhandle lubricating oil distillate can be carried out to provide a yield of lubricating oil of about 62 to 69%, while recovery of a similar quality lubricating oil from catalytically cracked products can only be achieved at yields of about 37 to 35 25%. Of equal importance is the fact that larger amounts of solvent must be used when extracting catalytically cracked products as shown by a lower raffinate productivity factor which will be defined subsequently. It is apparent from this that lubricating oils can only be

40 produced from catalytically cracked products in existing lubricant plants by loss in yield of the final lubricant product as compared to operation of the plant when employing a paraffinic base lubricating oil.

45 It is the particular object of this invention to provide a process for solvent extracting catalytically cracked products in order to obtain lubricating oils at higher yields for a given solvent extraction capacity and treat than heretofore obtainable. The process of this invention is based on the unexpected discovery that marked processing advantages are obtained by extracting mixtures of the lubricating oil fractions derived from cycle stock and derived from paraffinic base crude oils.

50 The nature of this process can be understood by reference to the accompanying drawing which diagrammatically illustrates a preferred embodiment of the present invention.

55 In accordance with the invention a paraffinic base crude oil is brought into a distillation zone 2 through line 3.

The distillation operation may be conducted to permit removal of light petroleum fractions through lines 4, 5, 6, and 7 and a lubricating oil fraction through line 8. Residual fractions of the petroleum oil may be removed as a bottoms product through line 9. While distillation zone 2 is shown as a single zone, it is understood that it may comprise a plurality of zones operating at different pressures if desired.

The waxy lubricating oil fraction withdrawn from still 2 through line 8 will constitute a portion of the original crude oil and will boil within the range of about 650 to 1100° F. It will normally have a dewaxed viscosity index of about 70 to 90. In the practice of this invention this lubricating oil fraction is processed in combination with a cycle oil derived from a catalytic cracking operation as indicated in the lower portion of the drawing.

A crude petroleum oil such as a mixed base crude oil is introduced to distillation zone 10 through line 11. The distillation operation may be conducted to permit removal of volatile fractions overhead through line 13 and of heavier boiling products such as gasoline, kerosene and heating oils through side stream withdrawals 14, 15, and 16. A heavy boiling fraction boiling within the range of about 650 to 1100° F. may be withdrawn through line 17, with residual portions of the crude oil being withdrawn from still 10 through line 18. The fraction of stream 17 constitutes a gas oil which is subjected to catalytic cracking in zone 19.

The cracking operation to be carried out in zone 19 may be of any desired type. The catalyst employed may be a modified natural or synthetic clay or may constitute a gel type of catalyst. Examples of these are montmorillonite clays, silica-alumina, silica-magnesia composites or other conventional cracking catalysts. The operation may be of a continuous or batch nature employing fixed beds, moving beds, fluidized, or suspensoid systems. The heat required for cracking may be supplied as preheat of processed materials and/or as the sensible heat of exothermically regenerated catalyst or in any other conventional manner. The cracking is carried out at temperatures of about 800 to 1000° F. and pressures of about atmospheric to 25 p. s. i. g. or higher in a manner which is well known.

The total cracked products are removed from cracking zone 19 through line 20 and are conducted to a product fractionator 21. Fractionator 21 may be operated to remove lighter fractions of the cracked products through overhead line 22 and side-stream withdrawals 23, 24, and 25. A bottoms product is obtained from fractionator 21 through line 26. The bottoms product may include all portions of the catalytically cracked products boiling above about 650° F. and in the event the cracking operation was of a fluidized nature this product may include a small amount of catalyst particles carried over from the catalytic cracking zone. In this case it is necessary to pass the product stream of line 26 to a separation zone 27 permitting separation of catalyst particles from the hydrocarbon product stream. Zone 27 may constitute a filtration zone or other means to separate the catalyst. The clarified product withdrawn from separation zone 27 is commonly called clarified oil or cycle oil. As used herein either of these terms is employed to identify the fraction of catalytically cracked products boiling within the range of about 650 to 1100° F.

In the practice of this invention, the cycle oil stream of line 28 and the virgin lubricating oil distillate stream of line 8 are combined and passed in admixture to dewaxing zone 30. The dewaxing operation carried out in zone 30 may be any of those conventionally used. In general, however, it is preferred that a solvent dewaxing operation be employed. For example, the hydrocarbon mixture supplied to zone 30 may be diluted with about 1 to 4 parts per volume of a solvent such as propane or methyl ethyl ketone. This mixture of hydrocarbon oil

and solvent is then heated sufficiently to secure the solution of all wax present. Thereafter, the mixture of oil and solvent is cooled to a temperature of about 25° F. to -50° F. so as to secure the crystallization of the wax present. The chilled mixture of oil, solvent and wax is then filtered to eliminate this wax permitting removal from zone 30 through line 31 of a dewaxed hydrocarbon oil.

The dewaxed oil is then passed through line 31 to a solvent extraction zone 32 wherein the oil is subjected to contact with a solvent exerting a selective solvent action towards aromatic constituents. As is well known, a variety of solvents may be employed to secure the desired selective removal of aromatic constituents. Thus, for example, sulfur dioxide, phenol, furfural, nitrobenzene, and other solvents may be employed. While the contacting of the solvent and oil may be conducted in any desired contacting equipment of a batch or continuous nature, countercurrent treating technique of the nature illustrated is preferably employed. In this technique the oil feed of line 31 is introduced to a countercurrent treating tower 32 at a point near the bottom thereof. Tower 32 may be provided with packing, perforated plates or equivalent means to secure effective liquid-liquid contact. A solvent such as phenol is brought into an upper portion of the tower through line 33. The oil passes upwardly through the tower while the solvent passes downwardly through the tower permitting removal from the bottom of the tower of the extract phase which is removed through line 33a. The material withdrawn from the top of tower 32 through line 34 is known as the raffinate phase and consists principally of the initial oil feed minus the major amount of the aromatic constituents originally present in the feed, admixed with small proportions of the solvent employed during the contacting.

The particular details relating to the solvent extraction step are not a part of this invention and it is to be understood that any desired refinements of solvent extraction operations may be used. For example, when employing phenol as a solvent it is preferred to employ about 0 to 10% of water as a solvent modifier. Again, it is ordinarily preferred to maintain a temperature gradient along the solvent extraction tower so that the bottom of the tower will ordinarily be maintained at a temperature of about 150 to 250° F. while the top of the tower will be maintained at a temperature of about 160 to 260° F. While the amount of solvent required will depend upon the properties of the oil feed and the desired properties of the raffinate product, in general, about 100 to 400% of solvent is employed, based on the oil feed.

The raffinate product of line 34 is preferably passed to a final distillation zone 35 wherein residual solvent is driven overhead through line 36 while the final lubricating oil product is removed as a bottoms product through line 37. It will also be understood that the lube product of line 37 may be subjected to other finishing operations such as clay treating or the like.

In the process particularly illustrated in the drawing, it was indicated that the cycle oil and virgin lube distillate were to be dewaxed prior to the solvent extraction operation. This is an optional feature since, if desired, the two distillates can first be solvent extracted and the raffinate of this operation can be subjected to dewaxing. Again, while the process illustrated applies a dewaxing operation to a mixture of the virgin lube distillate and the cycle oil lube distillate, it is to be understood that if desired these two distillates could be separately dewaxed. The essential feature of the process illustrated is the combination of these distillates during the solvent extraction step of the operation described.

In order to demonstrate the utility of this invention, reference will be made to exemplary data showing the advantageous features of the inventive process. In a first series of experiments a 150 neutral distillate was separated from a cycle oil derived from catalytic crack-

ing and a 150 neutral distillate was segregated from a Panhandle crude oil. These two dewaxed distillates were separately and in admixture subjected to solvent extraction. The conditions of solvent extraction were carefully adjusted so as to secure lubricating oil raffinate products having substantially the same viscosity index in all cases. Table I hereafter summarizes all pertinent data relating to these experiments:

TABLE I  
Phenol extracting Panhandle and cycle stock mixture of dewaxed 150 neutral

|                                 | Panhandle | 50% Panhandle, 50% Cycle Stock | Cycle Stock |    |
|---------------------------------|-----------|--------------------------------|-------------|----|
| Charge Stock Source:            |           |                                |             |    |
| Gravity, °API                   | 27.7      | 20.4                           | 12.2        |    |
| Flash, °F., COC                 | 415       | 410                            | 415         |    |
| Vis.:                           |           |                                |             |    |
| @ 100° F., SSU                  | 203       | 251                            | 412         |    |
| @ 210° F., SSU                  | 45.7      | 46.7                           | 49.7        |    |
| V. I.                           | 83        | 56                             | 0           |    |
| Pour, °F.                       | 15        | 15                             | 5           |    |
| Treating Conditions:            |           |                                |             |    |
| Vol. Percent Phenol             | 175       | 141                            | 140         | 25 |
| Percent Water in Phenol         | 3.0       | 3.0                            | 3.0         |    |
| Percent Water Injected in Tower |           |                                |             |    |
| Bottom                          | 2.7       | 2.8                            | 3.0         |    |
| Tower Temp., °F.:               |           |                                |             |    |
| Top                             | 221       | 191                            | 163         |    |
| Bottom                          | 209       | 180                            | 156         |    |
| Raffinate:                      |           |                                |             |    |
| Yield, Vol. Percent             | 62        | 51                             | 37          | 30 |
| Gravity, °API                   | 33.0      | 32.9                           | 32.7        |    |
| Flash, °F., COC                 | 435       | 415                            | 425         |    |
| Vis.:                           |           |                                |             |    |
| @ 100° F., SSU                  | 148.0     | 148.0                          | 151.3       |    |
| @ 210° F., SSU                  | 43.7      | 43.7                           | 43.9        |    |
| V. I.                           | 113       | 113                            | 112         |    |
| Pour, °F.                       | 25        | 25                             | 20          | 35 |
| Extract:                        |           |                                |             |    |
| Yield, Vol. Percent             | 38        | 49                             | 63          |    |
| Gravity, °API                   | 19.8      | 9.4                            | 2.4         |    |
| Flash, °F., COC                 | 425       | 410                            | 420         |    |
| Vis.:                           |           |                                |             |    |
| @ 100° F., SSU                  | 400       | 726                            | 1,700       |    |
| @ 210° F., SSU                  | 51.0      | 54.7                           | 62.5        |    |
| V. I.                           | 30        | -56                            | -202        |    |
| Productivity Factor Y/T         | 0.35      | 0.36                           | 0.26        |    |

In the data presented in Table I, a factor called productivity factor or  $Y/T$  is employed. In this expression  $Y$  is the raffinate yield and  $T$  is the phenol treat required so that this expression serves to correlate the yield of lubricating oil obtained with the treat of solvent required. With reference to the solvent extraction of the Panhandle neutral distillate by itself, it will be observed that a productivity factor of 0.35 was obtained, in order to obtain a lubricating oil product having a viscosity index of 113. For comparative purposes, however, it will be observed that in extracting the cycle stock neutral distillate, a productivity factor of only 0.26 was obtainable producing a lubricating oil distillate having a viscosity index of 112. These data indicate that in the solvent extraction of lubricating oil feed stocks to provide lubricating oil having a viscosity index of about 112, a 35% greater  $Y/T$  is obtained when employing a Panhandle distillate feed stock as compared to the  $Y/T$  of a cycle stock distillate feed stock. However, as shown in Table I, provided a mixture of 50% of each of these dewaxed distillates is employed, a lubricating oil product can be obtained having the same viscosity index at a productivity factor substantially that when processing Panhandle distillate alone. Thus, in accordance with this invention it is possible to upgrade cycle stock to lubricating oil without the serious drop in yield-treat relationship which would ordinarily be sustained by extracting the cycle stock alone.

A second series of experiments were then conducted employing a somewhat heavier lubricating oil fraction of cycle stock and Panhandle crude oil. The complete data relating to these experiments are set forth in Table II:

6  
TABLE II  
Phenol extracting Panhandle and cycle stock mixture of dewaxed light motor oil

|                                 | Panhandle | 50% Panhandle, 50% Cycle Stock | Cycle Stock |
|---------------------------------|-----------|--------------------------------|-------------|
| 10 Charge Stock Source:         |           |                                |             |
| Gravity, °API                   | 26.2      | 16.1                           | 4.8         |
| Flash, °F., COC                 | 455       | 450                            | 480         |
| Vis.:                           |           |                                |             |
| @ 100° F., SSU                  | 426       | 863                            | 4,620       |
| @ 210° F., SSU                  | 57.1      | 66.1                           | 97.7        |
| V. I.                           | 83        | 32                             | -152        |
| Pour, °F.                       | 5         | -10                            | 5           |
| 15 Treating Conditions:         |           |                                |             |
| Vol. Percent Phenol             | 168       | 119                            | 124         |
| Percent Water in Phenol         | 3.0       | 3.0                            | 3.0         |
| Percent Water Injected in Tower |           |                                |             |
| Bottom                          | 2.8       | 2.9                            | 2.9         |
| Tower Temp., °F.:               |           |                                |             |
| Top                             | 219       | 192                            | 176         |
| Bottom                          | 210       | 180                            | 166         |
| 20 Raffinate:                   |           |                                |             |
| Yield, Vol. Percent             | 69        | 51                             | 25          |
| Gravity, °API                   | 30.8      | 30.7                           | 31.9        |
| Flash, °F., COC                 | 450       | 455                            | 470         |
| Vis.:                           |           |                                |             |
| @ 100° F., SSU                  | 298       | 299                            | 292         |
| @ 210° F., SSU                  | 53.3      | 53.5                           | 53.8        |
| V. I.                           | 105       | 106                            | 111         |
| Pour, °F.                       | 15        | 15                             | 15          |
| Extract:                        |           |                                |             |
| Yield, Vol. Percent             | 31        | 49                             | 75          |
| Gravity, °API                   | 1,6.7     | 3.4                            | -2.5        |
| Flash, °F., COC                 | 450       | 455                            | 475         |
| Vis.:                           |           |                                |             |
| @ 100° F., SSU                  | 1,689     | 126.8                          | 186         |
| @ 210° F., SSU                  | 80.2      | 126.8                          | 186         |
| V. I.                           | -4        | 0.41                           | 0.20        |
| Productivity Factor Y/T         | 0.41      | 0.43                           | 0.20        |

These data again bear out the very real advantages obtainable by solvent extracting mixtures of paraffinic lubricating oil distillate stocks and such distillates derived from catalytically cracked products. The yield-treat relationship in extracting this mixture of virgin lube distillate and cycle oil lube distillate is shown to be substantially that obtainable when extracting a paraffinic lube distillate alone, and substantially double that obtainable when extracting cycle oil alone.

As described, therefore, this invention concerns a process for manufacturing lubricating oils by solvent extraction of a mixture of a virgin lubricating oil distillate and a catalytic cycle oil. In order to obtain the benefits of this invention it is essential that the virgin lubricating oil distillate be obtained from a paraffinic base crude oil; such a distillate is particularly characterized by a viscosity index of about 70 to 90, based on the inspection of the dewaxed distillate. Substantially equal amounts of the cycle oil and virgin lubricating oil distillate are preferably employed. More broadly, however, the proportion of the cycle oil in the mixture may range from about 10% to 60%.

What is claimed is:

1. A combination process for producing lubricating oil comprising the steps of catalytically cracking a gas oil boiling within the range of about 650° to 1100° F., segregating a first oil fraction boiling within the range of about 650° to 1100° F. from the cracked products, segregating a second oil fraction boiling within the range of about 650° to 1100° F. from a paraffinic crude oil, and contacting a mixture of said first and second oil fractions with a selective solvent for aromatic compounds to remove aromatic compounds from the said mixture, said mixture containing about 50% of said first oil fraction, said process including the step of dewaxing said oil fractions.

2. A combination process for producing lubricating oil comprising the steps of catalytically cracking a gas oil boiling within the range of about 650° to 1100° F., segregating a first oil fraction boiling within the range of about 650° to 1100° F. from the cracked products, segregating a second oil fraction boiling within the range of

about 650° to 1100° F. from a paraffinic crude oil, and contacting a mixture of said first and second oil fractions with a selective solvent for aromatic compounds to remove aromatic compounds from the said mixture, said mixture containing about 10% to 60% of said first oil fraction, said process including the step of dewaxing said oil fractions.

## References Cited in the file of this patent

## UNITED STATES PATENTS

|           |                  |               |
|-----------|------------------|---------------|
| 2,017,432 | Bahlke           | Oct. 15, 1935 |
| 2,052,196 | Stratford        | Aug. 25, 1936 |
| 2,155,745 | Wagner et al.    | Apr. 25, 1939 |
| 2,228,510 | Dearborn et al.  | Jan. 14, 1941 |
| 2,281,894 | Von Fuchs et al. | May 5, 1942   |
| 2,660,552 | Blanding         | Nov. 24, 1953 |